

1,006,323.

L. E. WEMPLE.  
PROCESS OF REFINING LEAD AND LEAD ALLOYS.  
APPLICATION FILED JAN. 9, 1911.

Patented Oct. 17, 1911.



Attest  
C. J. McCormick  
E. B. Hansen.

Inventor:  
L. E. Wemple  
ATTY'S *Knight & Cook*  
BY *E. J. Knight*

# UNITED STATES PATENT OFFICE.

LELAND E. WEMPLE, OF ST. LOUIS, MISSOURI, ASSIGNOR OF ONE-HALF TO HOYT METAL COMPANY, OF ST. LOUIS, MISSOURI, A CORPORATION.

## PROCESS OF REFINING LEAD AND LEAD ALLOYS.

1,006,323.

Specification of Letters Patent. Patented Oct. 17, 1911.

Application filed January 9, 1911. Serial No. 601,511.

*To all whom it may concern:*

Be it known that I, LELAND E. WEMPLE, a citizen of the United States of America, residing at the city of St. Louis and State of Missouri, have invented certain new and useful Improvements in Processes of Refining Lead and Lead Alloys, of which the following is a full, clear, and exact description, reference being had to the accompanying drawing, forming a part of this specification.

My invention relates to a process for the removal of contaminating metals or foreign elements from pig lead and from alloys of lead and antimony, of lead and tin, and of lead antimony and tin, and particularly to the removal of arsenic antimony, or tin from lead; and to the removal of arsenic from antimonial lead or antimony-lead alloys, and from lead-tin-antimony alloys without the removal of either antimony or tin from the alloys.

While it is my intention by my process to provide for the removal from lead and lead alloys of the various impurities such as mentioned, the process is concerned greatly in the removal of arsenic from lead and particularly from what is commercially known as antimonial lead. The presence of arsenic in lead, and particularly antimonial lead, is extremely detrimental to the quality of the lead for various uses, and interferes with the use of antimonial lead for many alloys, being so detrimental that there is a material loss in price to the producer when any marked percentage of arsenic is present as compared with lead and antimonial lead, free, or substantially free, of arsenic. The arsenic that is to be found in antimonial lead occurs as an impurity in the ore from which the antimonial lead in the process of smelting and refining is finally produced and is sometimes found as an impurity in soft lead, but not in so large a percentage as in antimonial lead where it is nearly always present in some degree, and while its separation from antimonial lead has heretofore been possible in a laboratory, I am unaware of any practical process by which its removal has been possible in a commercial sense.

My process consists, generally speaking, in bringing the lead, or lead alloy, containing impurities, or foreign elements, such as those hereinbefore mentioned, while in a

molten state, in intimate contact with the hydroxid of an alkali, such as hydroxid of sodium, or hydroxid of potassium, whereby the foreign elements are attacked by said hydroxid while the metallic lead itself is 60 practically unattacked, and therefore remains in the metallic state, the contaminating metals undergoing a chemical change which I regard as oxidation or at least partial oxidation, combining with or becoming 65 held mechanically by the hydroxid.

My process may be carried out in the apparatus shown in the accompanying drawing, which is a longitudinal section of the apparatus.

In the drawing, A, B and C designate furnaces, preferably having individual fire-boxes a, b, and c. In the furnace A is a melting pot 1 having an outlet at its bottom, and having attached to it at such outlet a 75 discharge pipe 2, preferably provided with a cut off valve 3. In the furnace B and at a lower level than the level of the melting pot 1 is what I term a "reaction pot" 4, this pot being located beneath the discharge pipe 2. 80 5 is a discharge pipe leading from the bottom of the reaction pot and containing a trap 6. The pipe 5 leads to a point above a receiving pot 7 mounted in the furnace C and into which the purified lead is discharged after it has been treated for the purpose of refining it by the removal of the contaminating elements originally present therein.

8 designates a perforate pan or basin located above the reaction pot 4 and into which the molten lead falls as it is discharged from the melting pot 1 through the discharge pipe 2 and from which the molten lead in its impure state descends in 95 finely divided streams or drops into the reaction pot 4.

In carrying out my process in the use of the apparatus I have shown, the lead or lead alloy to be treated is melted in the 100 melting pot 1 and is discharged therefrom in a molten condition through the discharge pipe 2 so that it falls onto the basin 8 from which it passes in streams or drops into the reaction pot, as previously stated. The reaction pot contains a molten alkaline bath, for instance, either of sodium hydroxid or potassium hydroxid, and it is by the mingling of the lead with the alkaline substance in the reaction pot that the purification of 110

the lead is acquired. As the separation of the lead from its impurities takes place in the reaction pot, the lead by reason of its greater specific gravity as compared with the alkaline bath substance descends to the bottom of the reaction pot and escapes gradually from said pot through the trap 6 in the pipe 5 and through said pipe to the receiving pot 7. By causing the molten lead, 10 or lead alloys, as provided for in my apparatus to fall in finely divided condition into the alkaline bath in the reaction pot, provision is made for the contaminating metals being acted upon almost instantly by the 15 alkaline bath in said pot, with the result of more effectually causing such metals to combine with the alkaline bath substance and become freed from the lead or lead alloys which settle in the reaction pot in a practically pure condition following the separation 20 of the foreign elements therefrom.

I prefer to use in my process, sodium hydroxid, commonly known as caustic soda. It will be readily appreciated that inasmuch 25 as the metal treated by the process is of much higher specific gravity than the caustic soda, it quickly settles to the bottom after it has descended into the alkaline bath of caustic soda and is discharged from the 30 reaction pot through the trap 6 and the pipe 5 to the receiving pot 7. The trap just mentioned serves to retain by far the greater part of the caustic soda that is present with the metal at the bottom of the reaction pot, but 35 it will be apparent that some of the caustic soda will pass with the metal to the receiving pot. To provide for the removal of such alkaline refining substance, such as the caustic soda mentioned, from the lead after it has 40 passed into the receiving pot, I introduce into the receiving pot with the lead while still in its molten condition, a suitable neutralizing agent, the agent used being preferably anhydrous sodium hydrogen sulfate, or 45 commonly commercially termed niter-cake. After evaporating moisture from the niter-cake, I force pieces of it to the bottom of the receiving pot and it quickly melts and combines with the alkaline substance, in the 50 instance of the use of caustic soda forming sodium sulfate, which rises to the surface of the metal and is readily skimmed off. The moisture that is formed by the reaction under the conditions stated is converted by 55 the heat of the molten metal into vapor and this vapor by agitating the metal causes the caustic soda and nitercake to be brought into contact with each other.

The amount of alkaline substance used in 60 carrying out my process depends upon the depth of the alkaline bath required for the proper separation of the contaminating elements from lead or lead alloys, and upon the percentage of contaminating elements present in the lead or alloy. By continued use 65

of the alkaline bath substance, the virtues therein become exhausted, being converted into compounds with the foreign substances removed from the lead or alloy, and, therefore, the alkaline substance must be replenished from time to time. 70

My process, as first indicated, further contemplates the removal of arsenic from lead and lead alloys without the removal of antimony or tin, which it is desirable in many 75 instances to retain therein. In this connection, the process includes as an essential step the retardation of the action of the hydroxid of an alkali on the contaminating elements present in the lead, or lead alloy, 80 by the use of a reducing agent, which combines more or less with the hydroxid. As such reducing agent I would mention iron scale or iron filings, zinc dust, or aluminum powder. By the use of such retarding agent, 85 I provide for the removal from the product, of elements other than antimony and tin.

In case I desire by my process to remove arsenic only, from lead-antimony-alloys, lead-tin-alloys, or lead-tin antimony alloys 90 without removing the antimony or tin in the alloy, I prefer to use iron scale as the retarding agent, mixing preferably twenty (20) parts of iron scale into one hundred (100) 95 parts of hydroxid of an alkali in the reaction pot.

There are certain impurities that are acted upon more slowly than other impurities in carrying out my process of refining lead or lead alloys, and it is, therefore highly desirable to intensify the action of the refining agent to accelerate its action on such impurities. Of these impurities, I would mention particularly antimony, bismuth and tin. To facilitate and hasten the removal of these 100 metals from lead or lead alloys, I mix with the refining agent a suitable agent that will intensify the action on these metals. This intensifying agent may be, for example, sulfur, nitrate of sodium, peroxid of sodium, 105 nitrate of potassium, or chlorate of sodium.

While I have described as an essential element used as a refining agent in my process the hydroxid of an alkali, I desire it to be understood that there may be used with said 110 hydroxid any other substance it may be found desirable to use in carrying out the process. I further wish it understood that in making reference in this description and in the claims to the hydroxid of an alkali, 115 I include any equivalent for such hydroxid or any substance from which such hydroxid may be derived, as for instance, an oxid of an alkali.

I claim:

1. The process of refining lead or lead alloy, consisting in bringing the lead or lead alloy in a molten state into intimate contact in a suitable vessel with the hydroxid of an alkali, then withdrawing such lead or lead 120

125

130

alloy in a molten state from said vessel, and finally separating from the lead or lead alloy the alkali hydroxid carried therewith from said vessel by the introduction of a neutralizing agent.

2. The process of refining lead alloy, consisting in causing intimate contact between the lead alloy in a molten state and a refining agent, and retarding the action of the refining agent to provide for the retention in the lead alloy of a certain element present therein.

10 3. The process of refining lead alloy, consisting in causing intimate contact between the lead alloy in a molten state and a refining agent, and retarding the action of the refining agent by the introduction of a reducing agent, thereby providing for the retention of a certain element in the lead alloy.

20 4. The process of refining lead alloy con-

taining antimony and tin and other elements, consisting in causing intimate contact between the lead alloy, while in a molten state, and a refining agent, and mixing a reducing agent with the refining agent to retard the action of the refining agent, whereby the antimony and tin are caused to be retained in the alloy.

25 5. The process of refining lead alloy, consisting in causing intimate contact between the lead alloy, in a molten state, and the hydroxid of an alkali, or its equivalent, as a refining agent, and retarding the action of the refining agent to provide for the retention by the lead alloy of a certain element present therein.

LELAND E. WEMPLE.

In the presence of—

H. G. COOK,  
E. B. LINN.